# EUROPEAN PATENT SPECIFICATION

(11) **EP 1 586 688 B1**
(45) Date of publication and mention of the grant of the patent: **08.11.2006**
(21) Application number: 04008922.9
(22) Date of filing: 15.04.2004
(51) Int. Cl.: D04H 3/07, D01G 25/00

(54) **Strechable high-loft-flat-tube structure from continuous filaments**
Dehnbare, voluminöse, flachrohrförmige Strukture aus endlosen Filamenten
Structure extensible et volumineuse de forme cylindrique aplatie réalisée à partir de filaments continus

(43) Date of publication of application: 19.10.2005
(73) Proprietor: V.F.T.Inc., Montebello 90640 (US)
(72) Inventor: Chien, Tomas Jung-Fu, Montebello, CA 90640 (US)
(74) Representative: Philipp, Matthias

(56) References cited:
- EP-A- 0 343 978
- WO-A-93/00464
- WO-A-98/37264
- WO-A-02/070806
- US-A- 3 492 185
- US-A- 3 515 621
- US-A- 3 747 162
- US-B1- 6 550 107

## Description

### Field of invention

This invention is concerned with improvement in fiberfill batts, sometimes referred to as batting, and processes whereby such improved batts with desirable uniformity, balanced tensile strength in all directions, stretchability, and high loft may be obtained.

### Description of related art

U.S. Patent No. 3747162 issued to Watson on 24 July 1973 discloses a conventional apparatus for producing a cross-lapped structure of crimped continuous filaments. This conventional apparatus includes a banding device, a threaded roll device, a series of air spreaders, a pair of delivery rolls, a pair of rolls, a chute, a pneumatic or hydraulic cylinder, and an apron.

A tow of some 30,000 adjacent crimped continuous filaments is delivered from a container (not numbered) to the banding device. From the banding device, the tow is delivered to the threaded roll device, where the crimped continuous filaments are de-registered. From the threaded roll, the crimped continuous filaments are delivered to the air spreaders, where air jets are used to spread the crimped continuous filaments to form a spread web. From the air spreaders, the spread web is delivered to the delivery rolls, about which the spread web makes an S-wrap. From the delivery rolls, the spread web is delivered to the pair of rolls, where the spread web makes an S-wrap. From the rolls, the spread web is delivered to the chute made of doors. The chute is oscillated via the pneumatic or hydraulic cylinder connected with one of the doors. From the chute, the spread web is laid onto the apron in the form of a roll-driven endless belt. The oscillated chute and the roll-driven endless belt together produce a cross-lapped structure of crimped continuous filament. In the use of this conventional apparatus, several problems have been encountered. Firstly, after leaving the chute, the spread web billows out transversely. This makes the spread web thinner towards its lateral edges.

Secondly, the chute is oscillated, i.e., the lower end of the chute is reciprocated between two dead ends.

The speed of the lower end of the chute reaches its minimum value, i.e., 0, at two end points of its travel, and reaches its maximum value at a midpoint between the end points. By doing so, the lower end of the chute stays longer at the end points than at the midpoint. Since the spread web is delivered at a constant rate, the chute releases more weight of less-extended crimped continuous filaments when reaching the end points than when reaching the midpoint. Hence the cross-lapped structure is thinner along a midline than along the two sides. Thirdly, since the speed of the lower edges of the doors is much greater than that of a point of the roll-driven endless belt, the cross-lapped intersect angle between layers of spread web is very small. In other words, the spread web from crimped continuous filaments actually extends substantially transverse to a longitudinal direction, or machine direction (MD), of the cross-lapped structure. Thus, little strength is provided in the machine direction of the cross-lapped structure. Furthermore, the cohesion between layers of spread web in the cross-lapped structure is poor, and they cannot adequately hold on to each other. The cross-lapped structure also exhibits poor dimensional stability, especially along the midline where the weight and thickness are lowest. Therefore, resin bonding, needle punching, or thermal bonding must be used to minimize these problems.

Further, the WO 93/00464 issued to Asselin on 7 January 1993 discloses a method for producing a semi-finished nonwoven product. It discloses a lap which has been folded by a spreading lapping machine, and then the lap is drawn into a drawing machine, so that the lap is arranged in two directions which are substantially symmetrical relative to the lengthwise direction of the drawn product. Asselin provides a lapped product similar to that of US Patent No. 3747162, and therefore has the same deficiency, namely, the nonuniformity of weight from midline to the two sides of the cross-lapped web.

In addition, US Patent No. 3515621 issued to Watson on 2 June, 1970 discloses a nonwoven fibrous product which has been cross-lapped by rotating a bonded striated web to form a cross-lapped material. It is related to a bonded nonwoven fabric with little thickness. The method for producing such fabric involves two distinct steps. First is forming a striated bonded thin web, and second is taking the thin web and cross-lapping it into multiple-layer material. However, Watson does not teach the spreading process involving feeding and spreading during the cross-lapping process under constant tension; therefore, such product with cross-lapping lacks strength in all directions, including machine directions (MD) and cross-machine directions (CD), and it is also without any advantage with regard to mechanical characteristics such as the ability to stretch, tensile strength, etc.

The present invention is therefore intended to obviate or at least alleviate these problems.

### Summary of the invention

The present invention provides a new machine and process to make a cross-lapped flat-tube structure or batting of crimped continuous filaments with optimum balance of tensile strength in all directions, especially in machine (MD) and cross-machine (CD) directions, with good stretch recovery properties, dimensional stability, and high loft, and overcomes the important deficiencies mentioned above in the prior art.

This invention uses crimped continuous filaments tow band wrapping at constant tension and speed around a batt-forming device which spreads, extends, and cross-laps this tow continuously to form a uniform batting having balanced tensile strength and to provide structural stability and stretch recovery properties. Uncrimped continuous filaments having extendible properties, such as elastic fibers or latent crimped fibers, etc., which can be spread, extended, and cross-lapped can also be used with this invention. By adjusting the traveling speed of the tow band wrapping around the batt-forming device and the spread belt surface speed in the spreading zone as described below as a spread ratio in the batt-forming device, the fiber orientation can achieve between a 10- and 70-degree angle, preferably a 30- to 60-degree angle, vs. the CD direction, and achieve a fiber orientation between cross-lapped layers of close to a 20-to 140-degree angle, preferably a 60- to 120-degree angle. As an example, when the traveling speed of the tow band wrapping around the batt-forming device and the spread ratio are optimized, the fiber orientation can be maintained at about a 45-degree angle vs. the CD direction, and the fiber orientation between cross-lapped layers at close to a 90-degree angle. This combination of fiber orientation in a spread flat-tube structure provides the best balance in MD and CD strength with a ratio of 1:1 so that there are essentially no weak spots in the cross-lapped flat-tube structure regardless of which direction the structure is pulled. The resulting cross-lapped flat-tube structure also exhibits excellent stretch recovery properties, dimensional stability, and high loft. Since the cross-lapped structure is formed from continuous filaments into an endless flat tube with good cohesion between individual fibers and between spread tow layers, one can use it directly without additional bonding process for insulated apparel, sleeping bags, bedding articles, and furniture applications, thus eliminating the deficiencies of the conventional cross-lapped batting made by the prior art mentioned above.

The advantage of wrapping the batt-forming device under constant tension and speed throughout the spreading, extending, and cross-lapping process eliminates the deficiency of the prior art of forming a web that is thinner along the midline than along the two sides and the weight uniformity problem, especially in the midline of the final batting. By adjusting the traveling speed of the feeding device and the spread ratio of the forming device, a complete balance of the tensile strength and stretchability in MD and CD directions can be achieved, hence eliminating the deficiencies of the prior art, which has poor tensile strength and dimensional stability in the MD, or longitudinal, direction. Also the need for resin bonding, needle punching, or thermal bonding to improve cohesion between layers in the conventional cross-lapped structure can be eliminated, resulting in a stretchable, softer, and thicker structure to improve the aesthetics and warmth of the sleeping bags, insulated apparel, etc. These aspects of the present invention may be used separately or in combination to solve deficiencies of the conventional cross-lapped structure.

Because of the unique fiber orientation achieved by this invention and the precision control of the batting width, the cross-lapped flat-tube structure maintains the strength advantage of the spun bonded fabric but with improved stretchability, loft, and softness vs. spun bonded fabric. No resin, or thermal bonding, or mechanical entanglement such as needle punching is required for the cross-lapped flat-tube structure of this invention. If desired, one can also use the above conventional bonding processes to even further increase the batting strength but with increased stiffness.

Because the cross-lapped structure by this invention is formed under pre-determined constant tension and precise mechanically controlled spreading, extending, and cross-lapping, the stress applied on each filament is similar. Once the cross-lapped structure is released from the spread belt and is delivered to the conveyor, it maintains its dimensional stability and uniformity in this relaxed state. This cross-lapped flat tube structure can be used for insulated apparel, sleeping bags, bedding, and furniture applications without further bonding steps such as resin bonding, needle punching, and thermal bonding with low-melting binder fiber, which normally reduce softness and/or loft. Due to the unique stretchability property of the cross-lapped flat tube structure of this invention, it can easily regenerate its loft and resiliency from compression during shipping and storage by slightly stretching or fluffing the final products.

Particularly useful when a stretchable cover fabric or shell fabric is used is the ability of the flat-tube structure of this invention to conform to the stretching of the fabric without deterioration. The conventional resin bonded, needle-punched, and thermally bonded batting or cross-lapped structure cannot provide this regeneration property because individual fibers and cross-lapped layers are bonded and locked with each other and are not free to separate from the compressed bonded structure.

The differences between the cross-lapped flat-tube structure of this invention and spun bonded fabric are significant. The present invention allows fiber orientation at a 45-degree angle vs. the CD direction and a 90-degree angle between cross-lapped layers of spread tow for balanced strength. The resulting structure can be used directly without bonding vs. spun bonded batting, which must be bonded to stabilize the structure. Hence the cross-lapped flat-tube structure of this invention is softer and provides higher loft. In addition, the continuous filaments used in this invention can be crimped as an option vs. no crimp for spun bonded filaments directly extruded from spinnerets, therefore exhibiting its stretch recovery properties. Spun bonded battings are limited to low fiber orientation angles, no crimp in each filament, and a rigidly bonded structure leading to rigid and low-loft nonwoven fabric or batting.

As will be described below, the unique design of the batt-forming device allows multiple numbers of tows of crimped continuous filaments to be simultaneously fed onto the feeding zone and subsequently to be spread in the spreading zone. If desired, each tow fed from a different feeding device can be different in fiber type, denier, fiber cross-section, and other variables, resulting in a heterogeneous batt in one single step by the present invention, whereas an expensive multiple-step process or complicated layering mechanism is required to achieve a similar composition by other methods. Almost any kind of fiber, such as nylon, polyester, polypropylene, and elastic fibers, just to name a few, can be used in this invention. There is no fiber denier limitation in this invention. Various cross-sections of fiber, for example, round, trilobal, tetralobal, etc., can be used with this invention. Other variables, such as fiber surface modification, additive in polymer, etc., to provide special properties or functions in the batting can be used with the present invention.

### Brief description of drawings

The present invention will be described through a detailed illustration of embodiments, referred to in the attached drawings.
- Figure 1: perspective view of the machine for producing a cross-lapped flat-tube structure from two tows of crimped continuous filaments according to the first embodiment of the present invention.
- Figure 2: front view of a batt-forming device used in the machine of Figure 1.
- Figures 3: and 4 front and side views of the components of a batt-forming device used in the machine of Figure 1.
- Figure 5: enlarged sectional view of a pinwheel between the conveyers of the feeding zone and the spreading zone as used in the machine of Figure 1.
- Figure 6: front view of a modified batt-forming device used in the machine of Figure 1.
- Figure 7: drawing of spreading step 1 of each tow of crimped continuous filaments at 0 second according to the first embodiment of the present invention.
- Figure 8: drawing of spreading step 2 of each tow of crimped continuous filaments at 8 seconds according to the first embodiment of the present invention.
- Figure 9: drawing of spreading step 3 of each tow of crimped continuous filaments at 16 seconds according to the first embodiment of the present invention.
- Figure 10: drawing of spreading step 4 of each tow of crimped continuous filaments at 24 seconds according to the first embodiment of the present invention.
- Figure 11: graphic demonstration of no filament orientation angle change with either two or four groups of conveyors in the batt-forming device.
- Figure 12: perspective view of a machine for producing a cross-lapped flat-tube structure from two tows of crimped continuous filaments which are separated into many small bundles of filaments according to the first embodiment of the present invention.
- Figure 13: illustration of using a wide tow band to make flat-tube structure with minimal or no cross-lapped marks with the present invention.
- Figure 14: illustration of usual tow band width to make flat-tube structure with the present invention.
- Figure 15: illustration of a flat-tube structure made by the present invention.
- Figure 16: illustration of a cross-lapped structure made by the conventional process.
- Figure 17: perspective view of a machine for producing a cross-lapped flat tube from a tow of crimped continuous filaments according to the second embodiment of the present invention.
- Figure 18: perspective view of a machine for producing a cross-lapped flat-tube structure from four tows of crimped continuous filaments according to the third embodiment of the present invention.
- Figure 19: perspective view of a machine for producing a cross-lapped flat-tube structure from multiple tows of crimped continuous filaments according to the fourth embodiment of the present invention.
- Figure 20: perspective view of a machine for producing a cross-lapped flat-tube structure from tows of crimped continuous filaments with batt-forming device moving upward instead of downward as shown in Figures 1, 17, 18-and 19.
- Figure 21: perspective view of a machine for producing a cross-lapped flat-tube structure from tows of crimped continuous filaments according to the fifth embodiment of the present invention.

### Detailed description of the invention

Referring to Figure 1, according to the first embodiment of the present invention, a machine and process for producing a cross-lapped flat-tube structure of crimped continuous filaments includes two separate feeding devices 2a and 2b located 180 degrees apart from one another; a spreading, extending, and cross-lapping device 4, which will be called the batt-forming device 4; and a conveying device 6. A tow 1 of crimped continuous filaments is fed from each of the feeding devices 2a and 2b to the batt-forming device 4, where the tow 1 is spread, extended, and cross-lapped. From the batt-forming device 4, a cross-lapped flat-tube structure of crimped continuous filaments is delivered to the conveying device 6 and subsequently to the windup equipment.

The feeding devices 2a and 2b each consist of a container 8a and 8b respectively in which the tow is stored and a series of rolls 10a and 10b respectively for spreading and feeding the tow 1 from the containers 8a and 8b to the batt-forming device 4. Although not shown, a mechanism is used to carry and drive the feeding devices 2a and 2b wrapping around the batt-forming device 4 continuously either in a clockwise or counter-clockwise direction for producing a continuous cross-lapped flat-tube structure of crimped continuous filaments. Such a mechanism is not shown since it is not the spirit or an essential part of the present invention.

Referring to Figures 2 to 5, the batt-forming device 4 includes two groups of pin-covered conveyors 12a and 12b, and two curved plates 14a and 14b between which the two groups of conveyors are arranged. The first group 12a is arranged near one edge of each of the plates 14a and 14b, and the second group 12b is arranged on the opposite edge of each of the plates 14a and 14b. Each group of the conveyors 12a and 12b extend a portion beyond the edges of plates 14a and 14b for engagement with the tows 1 of crimped continuous filaments, which are wrapped around the batt-forming device 4. As shown in Figures 3 and 4, 12a and 12b each consist of two groups of conveyors. A slower-moving conveyor is in the feeding zone located in the upper section of the batt-forming device 4, and a faster-moving conveyor in the spreading zone is located in the lower section of the batt-forming device 4. As shown in Figures 3 and 4, the conveyors in the upper section of the batt-forming device 4 within the feeding zone, indicated as Fca and Fcb, which comprise two separate but identical conveyors, are driven by rolls of slower but identical rotating speed in both 12a and 12b. Therefore, the surface speeds of conveyors in the feeding zone are identical at 12a and 12b. The advantage of the two separate conveyors in the feeding zone is to provide additional anchor points and supports of the engaged tow band in the feeding zone so that they can prevent a potential filament entanglement problem within the tow band during the engaging and transferring processes within the feeding zone. These two conveyors identified in each of Fca and Fcb respectively as shown have identical construction and surface speed, and the conveyors are parallel to each other. The conveyor belt surfaces are covered with coarse pins extended on the surfaces to provide enough friction to hold filaments of the tow 1 in place and transport them to the spreading zone. Because there are two conveyors for each side of the feeding zone, there are also two corresponding pin-wheels for each of La and Lb respectively at the bottom of each conveyor Fca and Fcb in the feeding zone in 12a and 12b having fine pins on the surface with surface speed faster than that of the conveyors in the feeding zone to pick up filaments from the respective conveyors as shown in Figures 3 and 4.

As the tow 1 of crimped continuous filaments is engaged by coarse pins on the conveyors Fca and Fcb in the feeding zone and moved downward at slow speed, filaments maintain their positions parallel to each other in the tow 1 without separation or spreading. When the leading edge of the tow 1 reaches the joining line between the bottom of Fca and Fcb and the pin-wheels La and Lb, the filaments in the leading edge of the tow 1 are caught by fine pins on the surface of the fast-rotating pin-wheels La and Lb.

Figure 5 shows that, because the surface speed of the pin-wheel La is faster than that of the conveyor Fca in the feeding zone, the filaments are caught and picked up from the tow band and are separated from the majority of the filaments in the tow 1, which is still being held by coarse pins on the conveyors in the feeding zone. In a continuous operation, the rest of the tow band is moved downward continuously by conveyors in the feeding zone toward the fast-moving pin-wheel La until all filaments are picked up. Since the pin-wheel La picks up filaments in sequence and at a faster speed, the filaments on pin-wheel La are also parallel to each other but are further apart. The resulting spread batt on pin-wheel La's surface is much thinner than the thickness of the original tow 1 fed onto the conveyors in the feeding zone. As the leading edge of the spread batt moving downward reaches the joining line between the pin-wheels La and Lb and the top of the conveyors Sca and Scb in the spreading zone, the filaments in the leading edge of the spread batt on pin-wheels La and Lb are caught by the finer pins on the surface of the even faster-moving conveyors Sca and Scb in the spreading zone. The conveyors Sca and Scb are different from the conveyors Fca and Fcb in the feeding zone, and each forms only a single wider conveyor. Once again, because the surface speed of the conveyors Sca and Scb in the spreading zone is faster than that of the pin-wheels La and Lb, the filaments are caught and picked up by finer pins on conveyors Sca and Scb in the spreading zone from the leading edge of the spread batt and are separated from the majority of the filaments in the spread batt which are still being held by fine pins on the pin-wheels La and Lb. In a continuous operation, the rest of the spread batt is moved downward continuously by pin-wheels La and Lb toward the faster-moving conveyors Sca and Scb in the spreading zone until all filaments are picked up by finer pins in conveyors Sca and Scb in the spreading zone. The resulting spread structure on conveyors Sca and Scb in the spreading zone is a uniform, thin batt of spread crimped continuous filaments which are parallel to each other.

The ratio of the surface speed of the conveyors Sca and Scb in the spreading zone to that in the feeding zone is defined as the spread ratio. The spread ratio determines the filament orientation angle and the cross-lapped layer angle, as will be described later. The surface speed of the pin-wheels La and Lb is faster than that of the conveyors Fca and Fcb in the feeding zone, but is slower than that of the conveyors Sca and Scb in the spreading zone. Since the pin-wheels La and Lb act as a separating wheel to separate filaments from the tow bundle and to transfer the resulting thinner batt to the conveyors Sca and Scb in the spreading zone for further spreading, the speed of the pin-wheels La and Lb does not change the spread ratio of the final product. However, the pin-wheel speed is adjusted based on the tow denier, crimp level, and cohesiveness of the filaments so that the filaments can be separated from the tow bundle without entanglement or damage for the uniform spreading operation.

In another aspect of the present invention, referring to Figure 6, the batt-forming device 4 consists of four groups of conveyors 12a, 12a-1, 12b, and 12b-1 instead of the two described above; each group has two conveyors in the feeding zone and one conveyor in the spreading zone. The composition of each group of conveyors in Figure 6 is identical to that described in Figure 2 identified as 12a and 12b. The components of these two additional groups of conveyors 12a-1 and 12b-1 are the same as those of 12a and 12b described in Figures 3 to 5 with the exception that 12a-1 and 12b-1 are opposite to each other but are located 90 degrees away from 12a and 12b respectively. Identical to that of 12a and 12b shown in Figure 3, 12a-1 and 12b-1 each has a group of pin-wheels La-1 and Lb-1 respectively in between the feeding zone and spreading zone. With these two additional groups of conveyors and wheels, the principle operation of the batt-forming device 4 is identical to that described above, but a wider flat-tube structure can be made evenly from a wider batt-forming device 4. Because the tow of crimped continuous filaments has very good cohesion between the filaments, it is difficult to separate the individual filaments from each other if the distance between the two conveyors in which the tow 1 is engaged is large. By reducing the distance between the two adjacent conveyors as illustrated in Figure 6, the filament cohesive force between the two supporting conveyors can be overcome by the spreading force asserted on the filaments. And as the filament cohesive force is overcome, the crimped continuous filaments can be spread evenly and smoothly, instead of sporadically, when cohesive force is overridden to form a uniform flat-tube structure. More detailed illustrations will be given below.

As the width of the batt-forming device 4 increases, further additional groups of conveyors can be installed evenly around the surfaces of the two curved plates 14a and 14b, to a total of 6, 8, 10, etc., groups of conveyors. There is no limitation to the number of groups of conveyors that can be used in the batt-forming device 4.

Referring to Figure 1, the conveying device 6 includes two rolls 16 and an endless belt 18 mounted on and driven by the rolls 16 for delivering the cross-lapped flat-tube structure produced by the batt-forming device 4.

The operation of the first embodiment of the present invention is described in Figure 1 in the following sequences.
(1) There are two separate feeding devices 2a and 2b located opposite to each other relative to the batt-forming device 4. In a continuous operation, a first portion of the tow 1 of crimped continuous filaments is delivered from the container 8a through feeding and spreading rolls 10a to conveyor 12a in the feeding zone. Soon after the first portion of the tow 1 is engaged with the moving conveyor 12a, it is transported downward at a speed slower than that of the tow 1 delivery speed from 10a. In an identical operation, and travelling in the same clockwise direction around the batt-forming device 4 simultaneously, a first portion of the tow 1 of crimped continuous filaments is delivered from container 8b through feeding and spreading rolls 10b to conveyor 12b in the feeding zone. Soon after the first portion of the tow 1 is engaged with moving conveyor 12b, it is transported downward at a speed slower than that of the tow 1 delivery speed from 10b.
   When the feeding device 2a is rotated 180 degrees clockwise in front of the batt-forming device 4, a second portion of the tow 1 of crimped continuous filaments is delivered from container 8a through feeding and spreading rolls 10a and is engaged with conveyor 12b in the feeding zone. In the meantime, the feeding device 2b is also rotated 180 degrees clockwise around the back of the batt-forming device 4, and a second portion of the tow 1 of crimped continuous filaments is delivered from container 8b through feeding and spreading rolls 10b to conveyor 12a in the feeding zone.
(2) The leading edge of the tow 1 of crimped continuous filaments at the bottom of the conveyors in the feeding zone is picked up by pin-wheels La and Lb respectively at faster surface speed. Therefore, filaments are being spread under tension and deposited onto conveyors in the spreading zone on both 12a and 12b having an even faster surface speed than La and Lb. As the tows 1 of crimped continuous filaments are delivered continuously from conveyors in the feeding zone of 12a and 12b, a continuous spread flat tube of continuous filaments is formed in conveyors in the spreading zone of 12a and 12b. By adjusting the ratio of the surface speed of the conveyors in the spreading zone to that in the feeding zone, which is expressed as the spread ratio, and adjusting the width of tow bands and the delivery speed of the tows 1 to the batt-forming device 4, one can change the basis weight of the flat-tube structure and the inclined angle A of the filaments relative to the CD direction as shown in Figure 1. Ideally, a 45-degree angle will provide equal tensile strength in MD and CD directions at a ratio close to 1:1 for best balance of tensile strength. The present invention can achieve such an ideal angle of 45 degrees. To meet the specific requirements of the end product, one can adjust the angle A between approximately 10 and 70 degrees to provide the desired tensile strength, stretchability, and loft.
(3) In a continuous rotating motion, the feeding device 2a is moving to the back of the batt-forming device 4 in Figure 1 or facing the curved plate 14b in Figure 2, while the feeding device 2b is moving to the front of the batt-forming device 4 in Figure 1 or facing the curved plate 14a in Figure 2. A third portion of the tow 1 of crimped continuous filaments is delivered from container 8a through feeding and spreading rolls 10a and is engaged with moving conveyor 12a in the feeding zone. Simultaneously, in an identical operation, a third portion of the tow 1 of crimped continuous filaments is delivered from container 8b through feeding and spreading rolls 10b and is engaged with moving conveyor 12b in the feeding zone. This process is repeated many times exactly as described in sequences (1), (2), and (3) above; therefore, a continuous flat-tube structure of spread crimped continuous filaments is formed in the batt-forming device 4 and subsequently delivered to conveyor device 6.

Referring to Figures 7 to 10 as the illustrations of one aspect of the present invention, two 0.25-meter-wide tows of crimped continuous filaments are delivered from 8a and 8b respectively, wrapping around a 2-meter-wide batt-forming device 4 at a speed of 0.25 meter per second, which is identical to that of the conveyor speed in the spreading zone. The conveyor speed in the feeding zone is 1/8 of that of the conveyors in the spreading zone, or 0.03125 meter per second, resulting in a spread ratio of 8. As shown in Figures 7 to 10, in every eight seconds, tows 1 delivered from containers 8a and 8b have traveled the distance of 2 meters between conveyors 12a and 12b, with Figure 7 showing the first 0 second of traveling, Figure 8 showing the 8^{th} second of traveling, Figure 9 showing the 16^{th} second of traveling, and Figure 10 showing the 24^{th} second of traveling. During this period, the first portions of the engaged tows 1 have been spread from 0.25 meter to 2 meters in the spreading zone. Because 8a and 8b are traveling in the same direction but are 180 degrees apart, each spread tow pattern is also the opposite and mirror image of the other. However, when the two spread tow patterns are super-imposed on each other as in the continuous operation involving two separate feeding devices in the present invention, a continuous flat tube of spread crimped continuous filaments, as shown in Figure 1, is formed continuously.

Referring to Figure 6 as another illustration of other aspects of the present invention using four groups of conveyors instead of two as described above, two 0.25-meter-wide tows 1 of crimped continuous filaments are delivered from 8a and 8b respectively, wrapping around a 2-meter-wide batt-forming device 4 at a speed of 0.25 meter per second, which is identical to that of the conveyor speed in the spreading zone. Since all four pin conveyors in the feeding zone are moving at the same speed and all four pin conveyors in the spreading zone are moving at the same but faster speed, the operation is the same as in the above illustration. For example, after 8 seconds, the first portion of tow 1 engaged with 12a in Figures 7 to 10 having a 2-meter-wide batt-forming device 4 has been spread from 0.25 meter to 2 meters in the spreading zone, forming a 45 degree filament orientation angle between 12a and 12b. But adding two more groups of pin conveyors 12a-1 and 12b-1 as in Figure 6, after 8 seconds, the engaged tow at 12a also has been spread from 0.25 meter to 2 meters in the spreading zone, and the engaged tow at 12b-1 is only spread from 0.25 meter to 1 meter in the spreading zone because tow 1 engaged with 12b-1 is 4 seconds late after engaging with 12a. Referring to Figure 11, when the tow 1 has been moved to the pin conveyor 12b-1 from the pin conveyor 12b, the tow 1 has been spread only half distance that the tow 1 has been moved to the pin conveyor 12a; however, the filament orientation A at both 12b-1 and 12a is still maintaining 45 degrees. Because of this time delay to reach 12b-1, the spread tow formation is the same whether 12b-1 is installed in the batt-forming device 4 or not. The same situation can be applied with 12a-1 relative to the spread tow formation. The advantage of the additional two groups of conveyors 12a-1 and 12b-1 as described previously is reducing the distance between engaging conveyors to override the cohesive force exhibited in the tow 1 of crimped continuous filaments so that uniform and smooth spreading can be achieved to form a uniform flat-tube structure. With a much wider batt-forming device to make a wider flat-tube structure, additional groups of conveyors in the feeding zone and the spreading zone are beneficial to overcome the cohesive force of the crimped continuous filaments for a successful spreading operation.

In yet another aspect of the present invention, referring to Figure 12, the two separate tows 1 being fed from containers 8a and 8b respectively have a different configuration compared to that shown in Figure 1. The tows 1 shown in Figure 1 and described in this embodiment are very uniform tow bands which can be characterized as having essentially the same thickness, density, and continuity across the width of the tow band. The resulting cross-lapped flat-tube structure is a homogeneous, uniform structure in appearance and in properties, having balanced tensile strength in all directions and providing structural stability and stretch recovery properties. However, the tow bands shown in Figure 12 are separated into many small bundles of filaments by an additional special device, such as separating guide pins or guide rolls in 10a and 10b respectively, before feeding them to the batt-forming device 4. The resulting bundles of filaments within the tow band are separated from each other with a definite gap between them, with the distance depending on the design of the separating device. These heterogeneous tow bands consisting of many small bundles of filaments and space in between them can form a heterogeneous cross-lapped flat-tube structure of crimped continuous filaments using the same machine and process of the present invention. The resulting heterogeneous cross-lapped flat-tube structure has essentially the same structure and characteristics, mainly having a balance of tensile strength in all directions and providing structural stability and stretch recovery properties with some exceptions. There are many empty spaces without filaments formed along each layer of the batt and many holes created within the cross-lapped structure, as shown in Figure 12. The resulting cross-lapped flat-tube structure has the appearance of a loosely woven structure in the form of mesh wire or fishing net, with many holes between filament cross-over points. This structure provides unique attributes, such as high air permeability through open holes for good breathability with low density, resiliency, and good support, which can be used as components to satisfy important requirements in mattress and furniture applications. This further demonstrates the flexibility and versatility of the present invention. This aspect of the present invention can be used singularly or in combination with other aspects of the present invention as described in all embodiments of the present invention.

In yet another aspect of the present invention, referring to Figures 13 and 14, there are no limitations on the denier, homogeneity, and width of the tow bands to be used with the present invention. Contrary to the aspect described above as illustrated in Figure 12, the present invention can also provide a very uniform flat-tube structure with very little or no cross-lapped marks as normally appear in a conventional cross-lapped structure described in prior art. Instead of using the usual thick and narrow tow band, a thin but wider tow band can be used to achieve a much more uniform flat-tube structure with essentially no cross-lapped marks between layers. For example, by using a tow band width of 75 cm (H) (as shown in Figure 13) instead of the usual 25 cm (h) (as shown in Figure 14) as described above for the feeding tow for the batt-forming device 4, one can minimize or eliminate the cross-lapped marks on the flat-tube structure. Because the feeding tow as shown in Figure 13 is three times wider, it will overlap three times in the feeding zone of the batt-forming device before reaching the spreading zone; hence, the marks on the over-lapped layers in the feeding zone are virtually eliminated compared to the obvious heavy marks appearing on the two adjacent thick and narrow tow bands. The resulting flat-tube structure from this wide tow band has essentially no cross-lapped marks. This further demonstrates the flexibility and versatility of the present invention.

The cross-lapped angle between the two cross-lapped layers is ideally 90 degrees for equal strength in MD and CD directions. Other cross-lapped layer angles can be achieved by this invention by adjusting the traveling speed of feeding devices 2a and 2b wrapping around the batt-forming device 4 and the spread ratio of the conveyor speeds between spreading zone and feeding zone. To meet the specific requirements of the end use, one can achieve the cross-lapped layer angles between about 20 and 140 degrees for specific desired tensile strength, stretchability, and loft. It is desirable that the spread tow leaves the batt-forming device 4 for the conveying device 6 when the section of the tow 1 between the first and second portions is at an appropriate angle from the section of the tow 1 between the second and third portions. The angle will determine the tensile strength ratio between MD and CD directions of the cross-lapped flat-tube structure.

There is a very important distinction between the spread cross-lapped flat-tube structure of the present invention compared to conventional cross-lapping batting by the process described in the prior art mentioned earlier. The flat tube of the present invention is an endless tube structure with very good uniformity throughout the entire structure, including edges and center, with dimensional stability, good stretchability, and high loft as shown in Figure 15, whereas the batt created by a conventional cross-lapping method is a folding-layer structure which has the appearance of fish scales which can be peeled off layer by layer as shown in Figure 16, with deficiencies of uniformity, poor cohesion between layers, poor balance ofMD and CD tensile strength, and inadequate dimensional stability.

As shown in Figure 1, the feeding devices 2a and 2b are located at identical height in the feeding zone relative to the batt-forming device 4, and they are separated by 180 degrees and rotate around the batt-forming device 4 in a clockwise direction. However, the feeding devices 2a and 2b can be at different heights in the feeding zone relative to the batt-forming device 4, be different degrees apart, and rotate in different directions around the batt-forming device 4. As long as both feeding devices are located above the dividing line between the feeding zone and spreading zone, a flat-tube structure from spread tow 1 of crimped continuous filaments can be produced by the present invention.

Referring to Figure 17, according to a second embodiment of the present invention, a machine and process for producing a cross-lapped flat-tube structure of crimped continuous filaments includes a single feeding device 2; a spreading, extending, and cross-lapping device 4, which will be called the batt-forming device 4; and a conveying device 6. A tow 1 of crimped continuous filaments is fed from the feeding device 2 to the batt-forming device 4, where the tow 1 is spread, extended, and cross-lapped. From the batt-forming device 4, a cross-lapped flat-tube structure of crimped continuous filaments is delivered to the conveying device 6.

The feeding device 2 consists of a container 8 in which the tow 1 is stored and a series of rolls 10 for spreading and feeding the tow 1 from the container 8 to the batt-forming device 4. Although not shown, a mechanism is used to carry and drive the feeding device 2 wrapping around the batt-forming device 4 continuously, either in a clockwise or counterclockwise direction for producing a continuous cross-lapped flat-tube structure of crimped continuous filaments.

The batt-forming device consists of two groups of pin-covered conveyors 12a and 12b and two curved plates as shown in Figures 2 to 4. The description of the composition and operation of the batt-forming device 4 is identical to that in the first embodiment of the present invention and is shown in Figures 2 to 4.

The operation of the second embodiment of the present invention is similar to that of the first embodiment of the present invention except a single container is needed as described as container 8a in the first embodiment of the present invention. The other exception is that the conveyor speed of 12a and 12b in the feeding zone is even slower than that of the tow delivery speed from the series of rolls 10, for example, 1/16 instead of 1/8, as in the case of the first embodiment. Because of the speed difference, a single feeding device can cover the total area needed for two feeding devices as shown in Figures 7 to 10. In order to keep a spread ratio of 8, the conveyor speed in the spreading zone is eight times faster than that of the conveyor speed in the feeding zone. As result, unlike the illustration in Figures 7 to 10, the tow 1 speed from container 8 wrapping around the batt-forming device 4 is actually twice (2x) that of the conveyor speed in the spreading zone. In other words, in eight seconds, container 8 has made one complete circle (360 degrees) around the batt-forming device 4 and engaged a third portion of the tow 1 with 12a instead of just traveling half a circle (or 180 degrees) or engaging a second portion of tow 1 with 12b. This illustrates the flexibility and versatility of this machine and process to make flat-tube structures with various basis weights, filaments and cross-lapped angles, and productivity by adjusting various combinations of the tow 1 denier, the feeding speed from container 8, and the spread ratio of the batt-forming device 4.

Referring to Figure 18, according to a third embodiment of the present invention, a machine and process for producing a cross-lapped flat-tube structure of crimped continuous filaments includes four separate feeding devices 2a and 2b located at the same height relative to the batt-forming device 4, both rotating in the same direction as shown in Figure 1, and 2c and 2d located at the same height but higher than that of 2a and 2b relative to the batt-forming device 4, both rotating in the same direction, which could be the same as or different from the direction of 2a and 2b.

As shown in Figure 18, 2a and 2b rotate clockwise around the batt-forming device 4 and both are located just above the dividing line between the feeding zone and the spreading zone. The other two feeding devices 2c and 2d rotate counter-clockwise around the batt-forming device 4 and are located higher above both 2a and 2b and also further away from the dividing line between the feeding zone and the spreading zone.

The procedure of engaging and spreading the tows 1 of crimped continuous filaments from containers 8a and 8b is identical to that of the three sequences (1), (2), and (3) described previously in the first embodiment of the present invention shown in Figure 1. The other two feeding devices 2c and 2d are located opposite to each other but above 2a and 2b relative to the batt-forming device 4. In a continuous operation, a first portion of the tow 1 of crimped continuous filaments is delivered from the container 8c through feeding and spreading rolls 10c to conveyor 12a in the feeding zone. Soon after the first portion of the tow 1 is engaged with the moving conveyor in the feeding zone 12a, the engaged portion of the tow 1 is being transported downward at a slower speed than that of the tow 1 delivery speed from 10c. Simultaneously in an identical operation, and traveling in the same counter-clockwise direction around the batt-forming device 4, a first portion of the tow 1 of crimped continuous filaments is delivered from container 8d through feeding and spreading rolls 10d to conveyor 12b in the feeding zone. Soon after the first portion of the tow 1 is engaged with the moving conveyor 12b in the feeding zone, the engaged portion of the tow 1 is being transported downward in similar fashion as the engaged tow 1 from container 8c. When feeding device 2c is rotated 180 degrees counterclockwise around the back of the batt-forming device 4, or facing the curved plate 14b in Figure 2, a second portion of the tow 1 of crimped continuous filaments is delivered from container 8c through feeding and spreading rolls 10c and is engaged with conveyor 12b in the feeding zone. In the meantime, the feeding device 2d is also rotated 180 degrees counterclockwise around the front of the batt-forming device 4 or facing the curved plate 14a in Figure 2, and a second portion of the tow 1 of crimped continuous filaments is delivered from container 8d through feeding and spreading rolls 10d and engaged with conveyor 12a in the feeding zone. The process is repeated with the third and fourth portions of tows 1 of crimped continuous filaments from feeding devices 2c and 2d and the process is repeated continuously.

The engaged tows 1 in the feeding zone delivered from containers 8c and 8d are transferred along the downward moving conveyors 12a and 12b in the feeding zone for a distance until they reach close to the dividing line of the feeding zone and spreading zone and are laid over and combined with tows 1 from feeding devices 2a and 2b.

The leading edges of the combined tows 1 of crimped continuous filaments at the bottom of the conveyors in the feeding zone are picked up by pin-wheels La and Lb, as shown in Figures 3 to 5, at faster surface speed. Therefore, filaments are being spread under tension and deposited onto conveyors 12a and 12b in the spreading zone, with both having faster surface speed than that of La and Lb. As the tows 1 of crimped continuous filaments are delivered continuously from conveyors 12a and 12b in the feeding zone, a continuous cross-lapped flat-tube of spread crimped continuous filaments is formed in conveyors in the spreading zone of 12a and 12b of the batt-forming device 4, and subsequently delivered to conveying device 6. This part of the spreading, extending, and cross-lapping process is identical to that described in the first embodiment of the present invention.

The locations of the feeding devices 2a and 2b can be at the same or different heights above the dividing line between the feeding zone and the spreading zone. They may rotate in the same or different direction either clockwise or counterclockwise around the batt-forming device 4. The locations of feeding devices 2c and 2d are higher than those of 2a and 2b but each can be at the same or different heights and rotate in the same or different directions around the batt-forming device 4. Once again, the ratio of surface speed of the conveyors in the spreading zone to that in the feeding zone is expressed as the spread ratio. The spread ratio determines the filament orientation angle vs. the CD direction and the cross-lapped angle between layers of the flat-tube structure.

Referring to Figure 19, according to a fourth embodiment of the present invention, a machine and process for producing a flat-tube structure of spread crimped continuous filaments includes two separate feeding devices 22a and 22b. Each consists of multiple containers 9a, 10a, and 11a in 22a, and 9b, 10b, and 11b in 22b; a spreading, extending and cross-lapping device 4, now called the batt-forming device 4 comprising a feeding zone and spreading zone, with composition identical to that in Figures 2 to 4, and a conveying device 6. The number of containers in feeding devices 22a and 22b varies from 2 to 100, depending on the denier and the width of the tow 1 in each container. A tow 1 of crimped continuous filaments is fed from each of the containers in feeding devices 22a and 22b to the batt-forming device 4 where the tow 1 is spread, extended and cross-lapped into a flat-tube structure and is finally delivered to conveying device 6. The batt-forming device 4 and conveying device 6 in Figure 19 are identical to that in Figures 1 and 18. The mechanism of spreading, extending and cross-lapping according to this embodiment of the present invention is the same as described in Figure 1, except multiple numbers of tows 1 are fed to the batt-forming device 4 from each of the feeding devices 22a and 22b.

More than two additional feeding devices as described as 22a and 22b in Figure 18 can be used with the present invention to make various basis weights and compositions of the flat-tube structure.

To illustrate the flexibility and versatility of the present invention, referring to Figure 20, a feeding mechanism can consist of a track circle around the batt-forming device 4, which is fed by feeding devices 2 moving around the track at a pre-determined speed. If desired, for convenience, as shown in Figure 20, the conveyors in the batt-forming device 4 can move upward instead of downward as shown in Figure 1, so that the conveyors in the feeding zone are at the lower level and the conveyors in the spreading zone are at the upper level. As a result, the conveying device 6 and windup rolls 61 are also located at the higher level of the machine. The composition of the batt-forming device 4 is identical to that in Figure 1 with the same components as in Figures 2 to 4, except the conveyors in the feeding zone and the spreading zone are moving upward instead of downward. The principle of spreading, extending, and cross-lapping is exactly the same as that of the first embodiment of the present invention.

Referring to Figure 21, according to a fifth embodiment of the present invention, a commercially feasible and economically viable machine and process for producing a flat-tube structure of spread tow 1 of crimped continuous filaments includes a system composed of a batt-forming device 4, a conveying device 6, and a windup device 61, all connected to a rotating platform, and two or more stationary feeding devices 2. The composition of the batt-forming device 4 is identical to that in Figure 1, with the same components as in Figures 2 to 4, except the conveyors in the feeding zone and spreading zone are moving upward instead of moving downward. The principle of spreading, extending, and cross-lapping is exactly the same as that of the first embodiment of the present invention. As the platform rotates in either a clockwise or counterclockwise direction at a pre-determined speed, tows 1 of crimped continuous filaments are fed from stationary feeding devices 2 wrapping around the conveyors in the feeding zone at the lower level of the rotating batt-forming device 4. These engaged tows 1 are then spread in the spreading zone on the upper level and subsequently delivered to conveying device 6, followed by windup device 61. The ratio of the surface speed of the conveyors in the spread zone to that in the feeding zone is expressed as the spread ratio. Once again, the basis weight of the flat-tube structure, the angle between the filaments and the CD direction of the flat tube, and the cross-lapped angle between layers are determined by the combinations of the feeding speed of the tows, the width of the tow 1, and the spread ratio. The feeding devices 2 can be at the same level as shown in Figure 21, or in different platforms with various heights so that each tow 1 can be fed in different heights in the feeding zone of the batt-forming device 4. The number of containers in each feeding device 2 can vary from 2 to 100, depending on the denier and the width of the tow 1 in each container.

The rotating batt-forming device in Figure 21 can be driven by some other means other than the rotating platform as shown. The batt-forming device 4 also can be arranged in the same configuration as in Figure 1, where the conveyors in both the feeding zone and the spreading zone are moving downward, so that tows can be fed from the stationary feeding devices 2 to the feeding zone and transferred to the spreading zone one floor below. Subsequently, the spread flat tube is delivered to the conveying device 6 and windup unit 61 at the lower floor.

### Definition of terms:

A. Stretch recovery: A batting or nonwoven fabric is stretched to 150% to length L2 from the original length, Lo, and the stress is released. The recovery length, L1, is measured after 10 minutes' relaxation. The percent recovery, R, is calculated as: $R = \left\{1-( L 1 - Lo ) / \left(L2-Lo\right)\right\} \times 100$
   When L1 = L2, there is 0% recovery.
   When L1 = Lo, there is 100% recovery.
   The measurement is determined in both MD and CD directions of the sample. The higher the percent recovery, the better the stretchability.
B. Loft: Loft is defined as thickness per unit weight. For example, inch per oz. per square yard, or mm. per gram per square meter.
C. Dimensional stability: The ability to maintain the size, i.e., width, length and height, during processing and in use.
D. Tensile strength: The ability to withstand the stress applied on a sample without breaking.

### Examples

### Example 1

Referring to Figure 1, a tow 1 of crimped continuous filaments with 100,000 filaments and total denier of 600,000 having a width of 0.125 meter is fed from container 8a through a series of feeding and spreading rolls 10a which widen it to a 0.25-meter tow band, then wrap it clockwise around a 2-meter-wide batt- forming device 4 and engage it with conveyor 2a in the feeding zone at a speed equal to 0.25 meter per second. The feeding zone conveyor surface speed is about 0.03125 meter per second, which is about 1/8 of the feeding speed of the tow 1 wrapping around the batt-forming device 4. The tow 1 is spread by conveyor 12a in the spreading zone at a surface speed of 0.25 meter per second, resulting in a spread ratio of 8, which is equal to the conveyor surface speed in the spreading zone divided by the conveyor surface speed in the feeding zone. By the time the tow band travels 2 meters to reach and engage with conveyor 12b in the feeding zone, the first portion of the tow 1 at 12a has already been spread from 0.25 meters to 2 meters wide to form a batt with a 45-degree angle relative to the CD direction. Therefore, the original crimp in the continuous filaments is being extended, and the individual filaments in the tow 1 are spread and separated from each other. The first portion of the original 0.25-meter-wide tow band becomes a 2-meter spread and extended batt. Simultaneously, a second tow band of crimped continuous filaments with 100,000 filaments and total denier of 600,000 having a width of 0.25 meters is fed from container 8b through a series of feeding and spreading rolls 10b wrapping from the opposite position around the same 2-meter-wide batt-forming device 4 and engaged with conveyor 12b in the feeding zone at a speed equal to that of container 8a. A second spread, extended batt is formed similar to that of the first spread, extended batt. The two spread, extended batts form a cross-lapped structure with a cross-lapped angle about 90 degrees between the two batts. At this 90-degree angle, the cross-lapped structure has equal strength in both MD and CD directions, good stretch recovery properties, and high loft. In a continuous operation, these two tow bands from two separate feeding devices 8a and 8b make a continuous flat-tube structure as shown in Figure 13, with basis weight of about 100 grams per square meter. This flat-tube structure has layers wrapping around in continuous tubular form which cannot be peeled off, in contrast to the case of the conventional cross-lapped structure.

### Example 2

Referring to Figure 1, a tow 1 of crimped continuous filaments with 100,000 filaments and total denier of 600,000 as in Example 1 is fed to the batt-forming device 4 at the same speed as in Example 1. A second tow 1 is also identical to that of Example 1 and is fed to the batt-forming device 4 as described in Example 1. The only exception is that the spread ratio is 4 instead of 8 as in Example 1. The resulting spread flat-tube structure has filament orientation of about a 27-degree angle relative to the CD direction. The flat-tube structure has a cross-lapped angle between layers of about 54 degrees.

### Example 3

Referring to Figure 1, a tow 1 of crimped continuous filaments with 100,000 filaments and total denier of 600,000 as in Example 1 is fed to the batt-forming device at speed as in Example 1. A second tow 1 identical to that of Example 1 is fed to batt-forming device 4 as described in Example 1. The only exception is that the spread ratio is 12 instead of 8 as in Example 1. The resulting spread flat-tube structure has a filament orientation of about a 56-degree angle relative to the CD direction, and a cross-lapped angle between layers of about 112 degrees.

## Claims

1. A process for making a uniform cross-lapped flat-tube structure of crimped continuous filaments having almost not cross-lapped marks and layers that cannot be peeled off from the edges, and with optimum balance of tensile strength in all directions, good stretch recovery properties, dimensional stability, and high loft, forms a spread, extended, and cross-lapped flat-tube structure by feeding one or more tows (1) of crimped continuous filaments from one or a multiple number of feeding devices (2a)(2b) each consisting of one or a multiple number of containers under pre-determined constant tension and speed wrapping around a batt-forming device (4) having two or a multiple number of groups of pin conveyors, each conveyor consisting of two separate but identical slower-moving conveyors in the feeding zone located either in the upper or lower level of the batt-forming device (4), depending upon whether the tow-spreading movement is downward or upward, and a fast-moving conveyor which consists of a single wider conveyor in the spreading zone located either in the lower or upper level of the batt-forming device (4), depending upon whether the tow-spreading movement is downward or upward, a pin-wheel being located between the conveyors in the feeding zone and the conveyors in the spreading zone, continuously moving and spreading the tow either downward or upward, depending upon whether the tow spreading movement is downward or upward, with a spread ratio in the range of about 1:2 to 1:20, resulting in a uniform cross-lapped flat-tube structure having a filament orientation angle of about 10 to 70 degrees, preferably about 30 to 60 degrees, vs. the CD direction and a cross-lapped angle between cross-lapped layers of about 20 to 140 degrees, preferably at a 60- to 120-degree angle, delivering the structure to a conveyor (6) while the cross-lapped flat-tube structure dimensional stability is maintained.

2. A process, according to Claim 1, wherein one or more tows (1) of crimped continuous filaments are fed from a feeding device (2), and the tows (1) are wrapped around a batt-forming device (4) from the upper level of the feeding zone (Fca)(Fcb), and moving downward to the lower level of the spreading zone (Sca)(Scb).

3. A process, according to Claim 1, wherein two or more tows (1) of crimped continuous filaments are fed from two different feeding devices (2a)(2b), and the tows (1) are wrapped around a batt-forming device (4) from the upper level of the feeding zone (Fca)(Fcb), and moved downward to the lower level of the spreading zone (Sca)(Scb).

4. A process, according to Claim 1, wherein multiple numbers of tows (1) of crimped continuous filaments are fed from more than two feeding devices (2a)(2b), and the tows (1) are wrapped around a batt-forming device (4) from the upper level of the feeding zone (Fca)(Fcb), and moved downward to the lower level of the spreading zone (Sca)(Scb).

5. A process, according to Claim 1, wherein one or more tows (1) of crimped continuous filaments are fed from one or a multiple number of feeding devices (2a)(2b), and the tows (1) are wrapped around a batt-forming device (4) from the lower level of the feeding zone (Fca)(Fcb), and moved upward to the upper level of the spreading zone (Sca)(Scb).

6. A uniform cross-lapped flat-tube structure of crimped continuous filaments made according to Claim 1, 2, 3, 4 or 5, having almost no cross-lapped marks and layers that cannot be peeled off from the edges with a filament orientation angle of about 10 to 70 degrees, preferably about 30 to 60 degrees, vs. the CD direction of the flat tube, and a cross-lapped angle between cross-lapped layers of about 20 to 140 degrees, preferably about 60 to 120 degrees, with good balance of tensile strength in all directions, good stretch recovery properties, dimensional stability, and high loft.

7. A cross-lapped flat-tube structure, according to Claim 6, wherein a cross-lapped flat tube is subsequently bonded by needle punching, or resin spray and oven curing of the resin and thermal bonding, or other bonding methods to further stabilize and strengthen the structure.

8. A cross-lapped flat-tube structure, according to Claim 6, wherein a cross-lapped flat tube can achieve a much more uniform flat-tube structure with essentially no cross-lapped marks between layers by using a thin but wider tow (1) band instead of the usual thick and narrow tow (1) band; when the wider tow (1) band is fed to the batt-forming device (4), it will overlap many more times than usual in the feeding zone (Fca)(Fcb) before reaching the spreading zone (Sca)(Scb); hence, the marks on the over-lapped layers in the feeding zone (Fca)(Fcb) are virtually eliminated compared to the obvious heavy marks appearing on the two adjacent thick and narrow tow (1) bands.

9. A machine for making a uniform cross-lapped flat-tube structure of crimped continuous filaments having one or a multiple number of feeding devices (2a)(2b) which feed one or more tows (1) of crimped continuous filaments; each device (2a)(2b) consists of one or multiple containers (8a)(8b) under pre-determined constant tension and speed wrapping around a batt-forming device (4) having two or a multiple number of groups of pin conveyors (12a)(12b); each conveyor consists of two separate but identical slower-moving conveyors in the feeding zone located either in the upper or lower level of the batt-forming device (4), depending upon whether the tow-spreading movement is downward or upward, and a faster-moving conveyor which consists of a single wider conveyor in the spreading zone located either in the lower or upper level of the batt-forming device (4), depending upon whether the tow-spreading movement is downward or upward; pin-wheels (La)(Lb) are located between the conveyors (12a)(12b) in the feeding zone (Fca)(Fcb) and conveyors (12a)(12b) in the spreading zone (Sca)(Scb), and a conveying device (6) is located at the end of the machine for delivering the cross-lapped flat-tube structure produced by the batt-forming device (4).

10. A machine, according to Claim 9, wherein one or more tows (1) of crimped continuous filaments are fed from a feeding device (2), and each conveyor (12a)(12b) of a batt-forming device (4) consists of a separate but identical slower-moving conveyor in the feeding zone (Fca)(Fcb) located in the upper section of the batt-forming device (4), and a faster-moving conveyor which consists of a single wider conveyor in the spreading zone (Sca)(Scb) located in the lower section of the batt-forming device (4).

11. A machine, according to Claim 9, wherein two or more tows of crimped continuous filaments are fed from two different feeding devices (2a)(2b), and each conveyor (12a)(12b) of a batt-forming device (4) consists of a separate but identical slower-moving conveyor in the feeding zone (Fca)(Fcb) located in the upper section of the batt-forming device (4), and a faster-moving conveyor which consists of a single wider conveyor in the spreading zone located in the lower section of the batt-forming device (4).

12. A machine, according to Claim 9, wherein the multiple number of tows of crimped continuous filaments are fed from more than two feeding devices (2a)(2b), and each conveyor (12a)(12b) of a batt-forming device (4) consists of a separate but identical slower-moving conveyor in the feeding zone (Fca)(Fcb) located in the upper section of the batt-forming device (4), and a faster-moving conveyor which consists of a single wider conveyor in the spreading zone (Sca)(Scb) located in the lower section of the batt-forming device (4).

13. A machine, according to Claim 9, wherein the machine comprises a system composed of a batt-forming device (4), a conveying device (6), and a windup device (61) all connected to a rotating platform; one or a multiple number of tows (1) of crimped continuous filaments are fed from one or a multiple number of feeding devices (2), and each device consists of one or more containers (8) under pre-determined constant tension and speed wrapping around a batt-forming device (4) having two groups of pin conveyors (12a)(12b); each conveyor consists of a separate but identical slower-moving conveyors in the feeding zone (Fca)(Fcb) located in the lower section of the batt-forming device (4) and a faster-moving conveyor which consists of a single wider conveyor in the spreading zone (Sca)(Scb) located in the upper section of the batt-forming device (4); pin-wheels (La)(Lb) are located between the conveyors in the feeding zone (Fca)(Fcb) and conveyors in the spreading zone (Sca)(Scb), and a conveying device (6) is located at the end of the machine for delivering the cross-lapped flat-tube structure produced by the batt-forming device (4).

## Patentansprüche

1. Verfahren für die Herstellung einer einheitlichen kreuzweise überlappenden Flachrohrstruktur aus gecrimpten durchgehenden Filamenten, die nahezu keine kreuzweise überlappenden Markierungen aufweist und Schichten, die nicht von den Kanten abgewickelt werden können, mit einer optimalen Ausgewogenheit der Zugfestigkeit in alle Richtungen, guten Dehnungsrückformungseigenschaften, dimensionaler Stabilität und hohem Bauschvermögen; die eine gespreizte, erweiterte und kreuzweise überlappende Flachrohrstruktur bildet, indem eine oder mehrere Filamentstränge (1) aus gecrimpten durchgehenden Filamenten aus einer oder mehreren Zuführeinheiten (2a)(2b) zugeführt werden, wobei jede von ihnen aus einer oder mehreren Behältern besteht, die diese bei einer vorab festgelegten konstanten Spannung und Geschwindigkeit um eine fasermattenformende Baugruppe (4) wickeln, die zwei oder mehrere Gruppen von Stiftförderern aufweisen, wobei jeder Förderer aus zwei separaten aber identischen, sich langsamer bewegenden Förderern in der Zuführzone besteht, die sich entweder im oberen oder unteren Bereich der fasermattenformenden Baugruppe (4) befinden, abhängig davon, ob die strangverteilende Bewegung abwärts oder aufwärts erfolgt, und einem sich schnell bewegenden Förderer, der aus einem einzelnen breiteren Förderer in der Verteilerzone besteht und entweder im unteren oder oberen Bereich der fasermattenformenden Baugruppe (4) angeordnet ist, abhängig davon, ob die strangverteilende Bewegung abwärts oder aufwärts erfolgt, wobei ein Stiftrad zwischen den Förderern in der Zuführzone und den Förderern in der Verteilerzone positioniert ist, das den Strang kontinuierlich entweder abwärts oder aufwärts bewegt und verteilt, abhängig davon, ob die strangverteilende Bewegung abwärts oder aufwärts erfolgt, mit einer Verteilerrate von 1:2 bis 1:20, woraus eine gleichmäßige kreuzförmig überlappende Flachrohrstruktur entsteht, die einen Anordnungswinkel der Filamente von 10 bis 70 Grad aufweist, vorzugsweise zwischen 30 und 60 Grad, gegenüber der CD-Richtung, und einen kreuzweise überlappenden Winkel zwischen kreuzweise überlappenden Schichten von ungefähr 20 bis 140 Grad, vorzugsweise einen Winkel von 60 bis 120 Grad, wobei die Struktur an einen Förderer (6) weitergegeben wird, während die dimensionale Stabilität der kreuzweise überlappenden Flachrohrstruktur beibehalten wird.

2. Verfahren nach Anspruch 1, bei dem ein oder mehrere Stränge (1) aus gecrimpten durchgehenden Filamenten von einer Zuführeinheit (2) zugeführt werden und bei dem die Stränge (1) um eine fasermattenformende Baugruppe (4) gewickelt werden, aus dem oberen Bereich der Zuführzone (Fca)(Fcb) abwärts zur tiefer gelegenen Ebene der Verteilerzone (Sca)(Scb).

3. Verfahren nach Anspruch 1, bei dem ein oder mehrere Stränge (1) aus gecrimpten durchgehenden Filamenten von zwei unterschiedlichen Zuführeinheiten (2a)(2b) zugeführt werden und bei dem die Stränge (1) um eine fasermattenformende Baugruppe (4) gewickelt werden, aus dem oberen Bereich der Zuführzone (Fca)(Fcb) abwärts zur tiefer gelegenen Ebene der Verteilerzone (Sca)(Scb).

4. Verfahren nach Anspruch 1, bei dem mehrere Stränge (1) aus gecrimpten durchgehenden Filamenten von mehr als zwei unterschiedlichen Zuführeinheiten (2a)(2b) zugeführt werden und bei dem die Stränge (1) um eine fasermattenformende Baugruppe (4) gewickelt werden, aus dem oberen Bereich der Zuführzone (Fca)(Fcb) abwärts zur tiefer gelegenen Ebene der Verteilerzone (Sca)(Scb).

5. Verfahren nach Anspruch 1, bei dem ein oder mehrere Stränge (1) aus gecrimpten durchgehenden Filamenten von einer oder mehreren Zuführeinheiten (2a)(2b) zugeführt werden und bei dem die Stränge (1) um eine fasermattenformende Baugruppe (4) gewickelt werden, aus dem unteren Bereich der Zuführzone (Fca)(Fcb) aufwärts zur höher gelegenen Ebene der Verteilerzone (Sca)(Scb).

6. Eine einheitliche, kreuzweise überlappende Flachrohrstruktur, bestehend aus gecrimpten durchgehenden Filamenten, hergestellt entsprechend Anspruch 1, 2, 3, 4 oder 5, die nahezu keine kreuzweise überlappenden Markierungen aufweisen und Schichten, die nicht von den Kanten abgewickelt werden können, mit einem Filamentausrichtungswinkel von ungefähr 10 bis 70 Grad, vorzugsweise ungefähr zwischen 30 und 60 Grad, gegenüber der CD-Richtung des Flachrohres, und einem kreuzweise überlappenden Winkel zwischen kreuzweise überlappten Schichten von ungefähr 20 bis 140 Grad, vorzugsweise zwischen ungefähr 60 und 120 Grad, mit einer gut ausgeglichenen Zugfestigkeit in allen Richtungen, guten Dehnungsrückformungseigenschaften, dimensionaler Stabilität und hohem Bauschvermögen.

7. Eine kreuzweise überlappende Flachrohrstruktur in gemäß Anspruch 6, wobei ein kreuzweise überlappendes Flachrohr in der Folge durch Nadellochung oder ein Harzspray und Ofenhärtung des Harzes und thermische Bindung oder durch andere Bindungsmethoden zur weiteren Stabilisierung und Verstärkung der Struktur gebunden wird.

8. Eine kreuzweise überlappende Flachrohrstruktur gemäß Anspruch 6, wobei bei einem kreuzweise überlappenden Flachrohr eine sehr viel einheitlichere Flachrohrstruktur im Wesentlichen ohne kreuzweise überlappende Markierungen zwischen den Schichten erzielt werden kann, indem ein dünneres aber breiteres Strangband (1) statt des üblichen dicken und schmalen Strangbands (1) verwendet wird; wird das breitere Strangband (1) der fasermattenformenden Baugruppe (4) zugeführt, überlappt es wesentlich häufiger als üblich in der Zuführzone (Fca)(Fcb), bevor die Verteilerzone (Sca)(Scb) erreicht wird; folglich werden die Markierungen auf den überlappenden Schichten in der Zuführzone (Fca)(Fcb) im Vergleich zu den vorherigen offensichtlich starken Markierungen, die auf den beiden angrenzenden dicken und schmalen Strangbändern (1) vorliegen, nahezu vollständig beseitigt.

9. Vorrichtung zur Herstellung einer einheitlichen kreuzweise überlappenden Flachrohrstruktur, bestehend aus gecrimpten durchgehenden Filamenten, das über eine oder mehrere Zufuhreinheiten (2a)(2b) verfügt, die einen Strang oder mehrere Stränge (1) aus gecrimpten durchgehenden Filamenten zuführt; jede Einheit (2a)(2b) besteht aus einem oder mehreren Behältern (8a)(8b) und wickelt diese bei einer vorab festgelegten konstanten Spannung und Geschwindigkeit um eine fasermattenformende Baugruppe (4), die über eine oder mehrere Stiftförderergruppen (12a)(12b) verfügt; jeder Förderer besteht aus zwei separaten aber identischen, sich langsamer bewegenden Förderern in der Zuführzone, entweder im oberen oder unteren Bereich der fasermattenformenden Baugruppe (4), abhängig davon, ob die strangverteilende Bewegung abwärts oder aufwärts erfolgt, und einem sich schneller bewegenden Förderer, der aus einem einzelnen breiteren Förderer in der Verteilerzone besteht, der entweder im unteren oder oberen Bereich der fasermattenformenden Baugruppe (4) positioniert ist, abhängig davon, ob die strangformende Bewegung abwärts oder aufwärts erfolgt; wobei Stifträder (La)(Lb) zwischen den Förderern (12a)(12b) in der Zuführzone (Fca)(Fcb) und Förderern (12a)(12b) in der Verteilerzone (Sca)(Scb) positioniert sind und eine Fördereinheit (6) am Ende des Geräts angeordnet ist, um die kreuzweise überlappende Flachrohrstruktur, die durch die fasermattenformende Baugruppe (4) erzeugt wird, abzugeben.

10. Vorrichtung nach Anspruch 9, bei der ein oder mehrere Stränge (1) aus gecrimpten durchgehenden Filamenten von einer Zuführeinheit (2) zugeführt werden und jeder Förderer (12a)(12b) einer fasermattenformenden Baugruppe (4) aus einem separaten aber identischen, sich langsamer bewegenden Förderer in der Zuführzone (Fca)(Fcb) besteht, der sich im oberen Bereich der fasermattenformenden Baugruppe (4) befindet, und einem sich schneller bewegenden Förderer, der aus einem einzelnen breiteren Förderer in der Verteilerzone (Sca)(Scb) besteht, der im unteren Bereich der fasermattenformenden Baugruppe (4) angeordnet ist.

11. Vorrichtung nach Anspruch 9, bei der zwei oder mehrere Stränge (1) aus gecrimpten durchgehenden Filamenten von zwei verschiedenen Zuführeinheiten (2a)(2b) zugeführt werden und jeder Förderer (12a)(12b) einer fasermattenformenden Baugruppe (4) aus einem separaten aber identischen, sich langsamer bewegenden Förderer in der Zuführzone (Fca)(Fcb) besteht, der sich im oberen Bereich der fasermattenformenden Baugruppe (4) befindet, und einem sich schneller bewegenden Förderer, der aus einem einzelnen breiteren Förderer in der Verteilerzone besteht, der im unteren Bereich der fadenformenden Baugruppe (4) angeordnet ist.

12. Vorrichtung nach Anspruch 9, bei der mehrere Stränge aus gecrimpten durchgehenden Filamenten von mehr als zwei verschiedenen Zuführeinheiten (2a)(2b) zugeführt werden und jeder Förderer (12a)(12b) einer fasermattenformenden Baugruppe (4) aus einem separaten aber identischen, sich langsamer bewegenden Förderer in der Zuführzone (Fca)(Fcb) besteht, der sich im oberen Bereich der fäsermattenfbrmenden Baugruppe (4) befindet, und einem sich schneller bewegenden Förderer, der aus einem einzelnen breiteren Förderer in der Verteilerzone (Sca)(Scb) besteht, der im unteren Bereich der fadenformenden Baugruppe (4) angeordnet ist.

13. Vorrichtung nach Anspruch 9, die ein System umfasst, das aus einer fasermattenformenden Baugruppe (4), einer Fördereinheit (6) und einer Wickeleinheit (61) besteht, die alle mit einer rotierenden Plattform verbunden sind; wobei ein oder mehrere Stränge (1) aus gecrimpten durchgehenden Filamenten von einer oder mehreren Zuführeinheiten (2) zugeführt werden, wobei jede Einheit aus einem oder mehreren Behältern (8) unter einer vorab festgelegten konstanten Spannung und Geschwindigkeit, die um eine fasermattenformende Baugruppe (4) wickeln, besteht, die über zwei Stiftförderergruppen (12a)(12b) verfügt; jeder Förderer besteht aus einem separaten aber identischen, sich langsamer bewegenden Förderer in der Zuführzone (Fca)(Fcb), der sich im unteren Bereich der fasermattenformenden Baugruppe (4) befindet, und einem sich schneller bewegenden Förderer, der aus einem einzelnen breiteren Förderer in der Verteilerzone (Sca)(Scb) besteht, der im oberen Bereich der fasermattenformenden Baugruppe (4) angeordnet ist; Stifträder (La)(Lb) sind zwischen den Förderern in der Zuführzone (Fca)(Fcb) und der Verteilerzone (Sca)(Scb) positioniert, und eine Fördereinheit (6) ist am Ende der Vorrichtung ausgeführt und gibt die in der fasermattenformenden Baugruppe (4) erstellte kreuzförmig überlappende Flachrohrstruktur aus.

## Revendications

1. Procédé destiné à réaliser une structure de tube plat à chevauchement croisé uniforme constituée de filaments continus ondulés ne présentant presque aucune marque à chevauchement croisé et de couches qui ne peuvent pas être détachées des bords, et présentant un équilibre optimum entre la résistance à la traction dans toutes les directions, de bonnes propriétés de récupération après étirement, de stabilité dimensionnelle et de gonflant élevé, forme une structure de tube plat étalée, étendue et à chevauchement croisé en faisant avancer un ou plusieurs câbles (1) constitués de filaments continus ondulés à partir d'un dispositif d'avance, ou d'un nombre multiple de dispositifs d'avance (2a) (2b) constitués chacun d'un ou d'un nombre multiple de récipients sous une tension constante prédéterminée et enroulant en vitesse autour d'un dispositif de formation de nappage (4) comportant deux groupes de transporteurs à broches ou de multiples transporteurs à broches, chaque transporteur étant constitué de deux transporteurs séparés identiques se déplaçant plus lentement dans la zone d'avance situés soit dans le niveau supérieur, soit dans le niveau inférieur du dispositif de formation de nappage (4) selon que le mouvement d'étalement du câble se fait vers le bas ou vers le haut, et un transporteur se déplaçant rapidement, qui est constitué d'un seul transporteur plus large dans la zone d'étalement situé soit dans le niveau inférieur, soit dans le niveau supérieur du dispositif de formation de nappage (4) selon que le mouvement d'étalement du câble se fait vers le bas ou vers le haut, une roue à broche étant située entre les transporteurs dans la zone d'avance et les transporteurs dans la zone d'étalement, se déplaçant continuellement et étalant le câble soit vers le bas, soit vers le haut, selon que le mouvement d'étalement du câble se fait vers le bas ou vers le haut, avec un rapport d'étalement dans la plage d'environ 1 : 2 à 1 : 20, résultant en une structure de tube plat à chevauchement croisé uniforme présentant un angle d'orientation de filament d'environ 10 à 70 degrés, de préférence d'environ 30 à 60 degrés, par rapport à la direction CD et un angle de chevauchement croisé entre les couches à chevauchement croisé d'environ 20 à 140 degrés, de préférence à un angle de 60 à 120 degrés, en délivrant la structure à un transporteur (6) alors que la stabilité dimensionnelle de la structure de tube plat à chevauchement croisé est conservée.

2. Procédé selon la revendication 1, dans lequel un ou plusieurs câbles (1) constitués de filaments continus ondulés sont avancés depuis un dispositif d'avance (2) et les câbles (1) sont enroulés autour d'un dispositif de formation de nappage (4) depuis le niveau supérieur de la zone d'avance (Fca) (Fcb), et se déplaçant vers le bas jusqu'au niveau inférieur de la zone d'étalement (Sca) (Scb).

3. Procédé selon la revendication 1, dans lequel deux câbles ou plus (1) de filaments continus ondulés sont avancés depuis deux dispositifs d'avance différents (2a) (2b), et les câbles (1) sont enroulés autour d'un dispositif de formation de nappage (4) depuis le niveau supérieur de la zone d'avance (Fca) (Fcb), et déplacés vers le bas jusqu'au niveau inférieur de la zone d'étalement (Sca) (Scb).

4. Procédé selon la revendication 1, dans lequel de multiples nombres de câbles (1) de filaments continus ondulés sont avancés depuis plus de deux dispositifs d'avance (2a) (2b), et les câbles (1) sont enroulés autour d'un dispositif de formation de nappage (4) depuis le niveau supérieur de la zone d'avance (Fca) (Fcb), et déplacés vers le bas jusqu'au niveau inférieur de la zone d'étalement (Sca) (Scb).

5. Procédé selon la revendication 1, dans lequel un ou plusieurs câbles (1) constitués de filaments continus ondulés sont avancés depuis un ou un nombre multiple de dispositifs d'avance (2a) (2b), et les câbles (1) sont enroulés autour d'un dispositif de formation de nappage (4) depuis le niveau inférieur de la zone d'avance (Fca) (Fcb), et déplacés vers le haut jusqu'au niveau supérieur de la zone d'étalement (Sca) (Scb).

6. Structure de tube plat à chevauchement croisé uniforme constituée de filaments continus ondulés, réalisée selon la revendication 1, 2, 3, 4 ou 5 ne comportant pratiquement aucune marque de chevauchement croisé et des couches qui ne peuvent pas être détachées des bords avec un angle d'orientation de filaments d'environ 10 à 70 degrés, de préférence d'environ 30 à 60 degrés, par rapport à la direction CD du tube plat, et un angle de chevauchement croisé entre les couches à chevauchement croisé d'environ 20 à 140 degrés, de préférence d'environ 60 à 120 degrés, présentant un bon équilibre de résistance à la traction dans toutes les directions, de bonnes propriétés de récupération après étirement, de stabilité dimensionnelle et de gonflant élevé.

7. Structure de tube plat à chevauchement croisé selon la revendication 6, dans lequel un tube plat à chevauchement croisé est ensuite lié par aiguilletage, ou pulvérisation de résine et polymérisation au four de la résine et thermocollage, ou d'autres procédés de liaison pour stabiliser et renforcer davantage la structure.

8. Structure de tube plat à chevauchement croisé, selon la revendication 6, dans lequel un tube plat à chevauchement croisé peut obtenir une structure de tube plat beaucoup plus uniforme ne comportant pratiquement aucune marque de chevauchement croisé entre les couches en utilisant une bande de câble mince mais plus large (1) au lieu de la bande de câble épaisse et étroite (1) habituelle ; lorsque la bande de câble (1) plus large est avancée vers le dispositif de formation de nappage (4), elle recouvrira beaucoup plus de fois que d'habitude dans la zone d'avance (Fca) (Fcb) avant d'atteindre la zone d'étalement (Sca) (Scb) ; donc les marques sur les couches en chevauchement dans la zone d'avance (Fca) (Fcb) sont pratiquement éliminées par comparaison aux marques importantes évidentes apparaissant sur les deux bandes de câbles (1) épaisse et étroite adjacentes.

9. Machine destinée à réaliser une structure de tube plat à chevauchement croisé uniforme constituée de filaments continus ondulés comportant un ou un nombre multiple de dispositifs d'avance (2a) (2b) qui font avancer un ou plusieurs câbles (1) constitués de filaments continus ondulés ; chaque dispositif (2a) (2b) est constitué d'un ou de multiples récipients (8a) (8b) sous une tension constante et un enroulement à vitesse prédéterminés autour d'un dispositif de formation de nappage (4) comportant deux groupes de transporteurs à broches, ou un nombre multiple de groupes de transporteurs à broches (12a) (12b), chaque transporteur est constitué de deux transporteurs séparés mais identiques se déplaçant plus lentement dans la zone d'avance situés soit dans le niveau supérieur, soit dans le niveau inférieur du dispositif de formation de nappage (4) selon que le mouvement d'étalement de câble se fait vers le bas ou vers le haut, et un transporteur se déplaçant plus rapidement, qui est constitué d'un seul transporteur plus large dans la zone d'étalement situé soit dans le niveau inférieur, soit dans le niveau supérieur du dispositif de formation de nappage (4) selon que le mouvement d'étalement de câble se fait vers le bas ou vers le haut ; des roues à broches (La) (Lb) sont situées entre les transporteurs (12a) (12b) dans la zone d'avance (Fca) (Fcb) et les transporteurs (12a) (12b) dans la zone d'étalement (Sca) (Scb), et un dispositif de transport (6) est situé à l'extrémité de la machine destinée à délivrer la structure de tube plat à chevauchement croisé produite par le dispositif de formation de nappage (4).

10. Machine selon la revendication 9, dans laquelle un ou plusieurs câbles (1) constitués de filaments continus ondulés sont avancés depuis un dispositif d'avance (2) et chaque transporteur (12a) (12b) d'un dispositif de formation de nappage (4) est constitué d'un transporteur séparé mais identique se déplaçant plus lentement dans la zone d'avance (Fca) (Fcb) situé dans la section supérieure du dispositif de formation de nappage (4) et en un transporteur se déplaçant plus rapidement qui est constitué d'un transporteur unique plus large dans la zone d'étalement (Sca) (Scb) situé dans la section inférieure du dispositif de formation de nappage (4).

11. Machine selon la revendication 9, dans laquelle deux câbles constitués de filaments continus ondulés, ou plus, sont avancés depuis deux dispositifs d'avance différents (2a) (2b), et chaque transporteur (12a) (12b) d'un dispositif de formation de nappage (4) est constitué d'un transporteur séparé mais identique se déplaçant plus lentement dans la zone d'avance (Sca) (Scb) situé dans la section supérieure du dispositif de formation de nappage (4), et un transporteur se déplaçant plus rapidement, qui consiste en un seul transporteur plus large dans la zone d'étalement située dans la section inférieure du dispositif de formation de nappage (4).

12. Machine selon la revendication 9, dans laquelle le nombre multiple de câbles constitués de filaments continus ondulés sont avancés depuis plus de deux dispositifs d'avance (2a) (2b), et chaque transporteur (12a) (12b) d'un dispositif de formation de nappage (4) est constitué d'un transporteur séparé mais identique se déplaçant plus lentement dans la zone d'avance (Fca) (Fcb) situé dans la section supérieure du dispositif de formation de nappage (4) et un transporteur se déplaçant plus rapidement qui est constitué d'un seul transporteur plus large dans la zone d'étalement (Sca) (Scb) situé dans la section inférieure du dispositif de formation de nappage (4).

13. Machine selon la revendication 9, dans laquelle la machine comprend un système composé d'un dispositif de formation de nappage (4), d'un dispositif de transport (6) et d'un dispositif d'enroulement (61), tous reliés à une plate-forme tournante ; un câble ou un nombre multiple de câbles (1) constitués de filaments continus ondulés sont avancés depuis un dispositif ou un nombre multiple de dispositifs d'avance (2), et chaque dispositif est constitué d'un ou plusieurs récipients (8) sous une tension constante et un enroulement de vitesse prédéterminés autour d'un dispositif de formation de nappage (4) comportant deux groupes de transporteurs à broches (12a) (12b), chaque transporteur est constitué d'un transporteur séparé mais identique se déplaçant plus lentement dans la zone d'avance (Fca) (Fcb) situé dans la section inférieure du dispositif de formation de nappage (4) et d'un transporteur se déplaçant plus rapidement qui est constitué d'un seul transporteur plus large dans la zone d'étalement (Sca) (Scb) situé dans la section supérieure du dispositif de formation de nappage (4), des roues à broches (La) (Lb) sont situées entre les transporteurs dans la zone d'avance (Fca) (Fcb) et les transporteurs dans la zone d'étalement (Sca) (Scb) ainsi qu'un dispositif de transport (6) sont situés à l'extrémité de la machine destinée à délivrer la structure de tube plat en chevauchement croisé produite par le dispositif de formation de nappage (4).
